

# UNITED STATES PATENT OFFICE.

AXEL THEODOR CONSTANTIN ESTELLE, OF HAGEN, GERMANY, ASSIGNEE TO MARTIN  
FILIP WIJKSTROM, OF STOCKHOLM, SWEDEN.

## PROCESS OF ELECTROLYTICALLY PRODUCING IRON.

Specification of Letters Patent.

Patented Aug. 6, 1918.

1,275,161.

No Drawing.

Application filed November 22, 1916. Serial No. 132,768.

To all whom it may concern:

Be it known that I, AXEL THEODOR CONSTANTIN ESTELLE, a subject of the King of Sweden, residing at Hagen, in Westphalia, Germany, have invented a new and useful Process of Electrolytically Producing Iron, of which the following is a full, clear, and exact description.

My invention is directed to the production of iron by the electrolytic disassociation of a solution comprising a caustic alkali and a ferric hydrate.

A tank of iron or any other suitable material contains anodes and cathodes of iron or any other suitable material or the tank itself if built of conductive material may serve as an anode and contain said cathodes. The tank is filled with the electrolyte consisting of a hot slime of iron hydroxid and caustic soda or potash comprising for example 30% ferric hydrate, 35% caustic soda and 35% water. By the action of the electric current metallic iron is precipitated on the cathode in form of a smooth layer, and oxygen is developed near the anode, while the hydroxid is gradually decomposed. In order to render this process continuous, iron hydroxid may be added to the electrolyte in the electrolyzing tank or outside of it in proportion as metallic iron is precipitated. Instead of iron hydroxid most other compounds of iron with oxygen and hydrogen may be used. Iron compounds with oxygen alone are less appropriate for the process, but by a previous treatment with caustic or carbonic alkali at higher temperatures they may be rendered fit for it.

In carrying out my invention, I place the solution above described in one of the usual and well known devices usually employed in the electrolysis of metals and having the usual electrodes, which are initially preferably 30 mm. apart. A current which gives a potential difference of from 1.65 to 1.80 volts between the electrodes and a density of 3 amperes per square decimeter, has been found suitable at a temperature of 100° centigrade.

Some other metals, for instance cadmium, are equally precipitated by the electric cur-

rent from a slime, consisting of their oxids or hydroxids and caustic alkali solution; by mixing their compounds with the iron compounds the alloy of iron with these metals may be produced by this process. 55

Other metals, for instance nickel, are not precipitated under the same circumstances, and the process may therefore be used for separating iron from these metals.

When I speak in my claims of a caustic alkaline solution, I mean a solution comprising sodium hydroxid or potassium hydroxid, and when I speak of iron compounds comprising oxygen, I do not mean to include such as may not be suitable. 60

The above quantities, current strengths and temperatures are merely illustrative of my invention and changes may be made therein without departing from the scope of the appended claims. 70

I claim:

1. The process of electrolytically producing iron consisting in subjecting to electrolysis a slime of caustic alkaline solution and iron compounds comprising oxygen. 75

2. The process of electrolytically producing iron consisting in subjecting to electrolysis a slime of caustic alkaline solution and iron compounds comprising oxygen and hydrogen. 80

3. The process of electrolytically producing iron consisting in treating iron compounds with caustic or carbonic alkali at higher temperatures, and subjecting to electrolysis a slime of caustic alkaline solution 85 and said compounds.

4. The process of electrolytically producing iron consisting in treating iron oxids with caustic or carbonic alkali at higher temperatures, and subjecting to electrolysis a slime of caustic alkaline solution and said oxids. 90

5. The process of electrolytically producing iron consisting in subjecting to electrolysis a slime of caustic alkaline solution 95 and compounds containing iron and other metals, as for instance nickel, which cannot be precipitated by the electric current under the conditions of the process.

6. The process of electrolytically pro- 100

ducing alloys of iron with other metals consisting in subjecting to electrolysis a slime of caustic alkaline solution and a mixture of compounds of iron and of such metals, as for instance cadmium, which can be precipitated by the electric current under the conditions of the process.

In testimony whereof I have hereunto set my hand and seal in the presence of two subscribing witnesses.

AXEL THEODOR CONSTANTIN ESTELLE. [L. S.]

Witnesses:

WOLFRAM C. POECHER,  
AUGUST PESCH.